

# United States Patent

Shaw

[15] 3,635,769

[45] Jan. 18, 1972

[54] **NICKEL-CHROMIUM EUTECTIC ALLOY**

[72] Inventor: Bevill J. Shaw, Turtle Creek, Pa.

[73] Assignee: Westinghouse Electric Corporation, Pittsburgh, Pa.

[22] Filed: Aug. 21, 1969

[21] Appl. No.: 851,859

[52] U.S. Cl..... 148/32, 72/377, 75/171,  
75/176, 148/2, 148/3

[51] Int. Cl..... C22c 19/00

[58] Field of Search..... 75/171, 176, 134, 135, 122;  
148/2, 3, 4, 11.5, 133, 32, 32.5; 72/362, 377

[56]

References Cited

UNITED STATES PATENTS

3,124,452 3/1964 Kraft..... 75/134  
2,809,139 10/1957 Bloom et al..... 148/133

Primary Examiner—Richard O. Dean  
Attorney—F. Shapoe and Lee P. Johns

[57]

ABSTRACT

A nickel-chromium alloy consisting of about 50 percent of nickel and 50 percent of chromium and having an oriented lamellar microstructure which is obtained by directional solidification.

4 Claims, 7 Drawing Figures



PATENTED JAN 18 1972

3,635,769

SHEET 1 OF 4



FIG. I.

WITNESSES

Theodore F. Wrobel  
Loy M. Garman

INVENTOR

Bevil J. Shaw  
BY Lee P. Johnson  
ATTORNEY

PATENTED JAN 18 1972

3,635,769

SHOOT 2 OF 4

FIG. 2.



FIG. 6.



FIG.3.



FIG.4.



FIG. 5.



FIG. 7.

## NICKEL-CHROMIUM EUTECTIC ALLOY

## BACKGROUND OF THE INVENTION

## 1. Field of the Invention

This invention relates to a nickel-chromium eutectic alloy and, more particularly, it pertains to members of such an alloy having an oriented lamellar structure.

## 2. Description of the Prior Art

Increases in the efficiency of gas turbines are directly related to the properties of the material of which the turbine blades are composed. Small increases in operating temperature at the blade surface have always resulted in improved output for a given size of turbine. Thus the turbine blades are both the key to higher efficiency as well as a serious impediment to future improvements. That is true whether the turbine is designed for use in an aircraft, or in surface-based gas turbines which latter are frequently used to generate domestic electric power during peak demand hours or for standby use.

In those applications efficiency is not the only parameter of importance. An economically valid test of power-generating turbine systems is the service-free lifetime and the number of hours the unit may be operated on an intermittent duty cycle without reblading. For aircraft engines the turbine blades are used for up to 2,000 hours as compared with surface-based turbines which operate up to 10,000 hours without a service shutdown.

Related to the foregoing is the problem of corrosion resistance which governs the service life of turbine blades and particularly land-based turbines where a wide variety of corroding ambients are prevalent. Various so-called "super alloys," such as nickel- and cobalt-base alloys, have practically dominated all turbine blade applications heretofore. However, the chemical complexity of the alloys has resulted in many reactions which are not understood and are difficult to control. Overaging, for one reason, causes deterioration of mechanical properties after exposure at high temperatures and stresses. Precipitation of undesirable properties such as the sigma phase and grain boundary carbides is frequency detrimental to alloy performance and to longtime dimensional stability. Moreover, the metallurgical art which has optimized the mechanical performance of the alloys does not provide any base upon which to gauge corrosion resistance.

In the past it has been found that at least 12 percent chromium in nickel-chromium alloys was necessary to give fair corrosion resistance at high temperatures. Although the mechanical properties of this alloy are improved, as the percentage of chromium is reduced the corrosion resistance is lessened.

None of the prior existing alloys used for gas turbine blades have completely satisfied the threefold problems of thermal stability, strength, and corrosion resistance at elevated temperatures of operation.

Lamellar eutectic alloys as such are known: see U.S. Pat. No. 3,124,452 and an article entitled "Coarsening of Eutectic Microstructures at Elevated Temperatures" by L. D. Graham and R. W. Kraft on pages 94 to 101 of Vol. 236, Jan. 1966, issue of "Transactions of the Metallurgical Society of AIME."

## SUMMARY OF THE INVENTION

It has been found in accordance with this invention that the foregoing problems may be overcome by providing a nickel-chromium alloy consisting of about 50 percent nickel and 50 percent chromium and having an oriented lamellar microstructure. The nickel-chromium alloy of the present invention consists of a binary eutectic alloy of nickel and chromium which is substantially devoid of any intentional additional alloy elements and which may include only incidental impurities.

Accordingly, it is a general object of this invention to satisfy the foregoing problem by providing a nickel-chromium binary eutectic alloy having oriented lamellar microstructure.

It is another object of this invention to provide members of a nickel-chromium binary eutectic alloy consisting of 50 percent nickel and 50 percent chromium and which is substan-

tially devoid of additional elements, and has an oriented lamellar microstructure.

Finally, it is an object of this invention to satisfy the foregoing objects and desiderata in a simple and expedient manner.

## BRIEF DESCRIPTION OF THE DRAWINGS

For a better understanding of the invention reference is made to the accompanying drawings, in which:

5 FIG. 1 is a phase diagram of the nickel-chromium binary system;

10 FIG. 2 is a photomicrograph of a transverse section of a nickel-chromium eutectic alloy having oriented lamellae produced by unidirectional solidification (X150);

15 FIG. 3 is a graph of yield strength plotted as a function of  $d^{-1/2}$ , where  $d$  is the specimen diameter as a result of cold swaging of Ni-Cr eutectic alloy at room temperatures;

20 FIG. 4 is a bar chart showing the thermal stability of the Ni-Cr eutectic alloy at room temperature and at 1,400° F. both in the worked and unworked condition as compared with another nickel base alloy superalloy (René' 41);

25 FIG. 5 is a graph showing the creep-rupture behavior of Ni-Cr eutectic alloy at 760° C. in which specimens having a fully lamellar structure are compared with specimens having a partially lamellar structure;

30 FIG. 6 is a graph showing creep-rupture tests of the Ni-Cr eutectic alloy at 1,400° F. compared with 60 percent Cr-40 percent N: (high- and low-carbon) alloys; and

35 FIG. 7 is a graph showing the corrosion resistance of Ni-Cr eutectic alloy as compared with other high-temperature materials which have been used previously as gas turbine blades.

## DESCRIPTION OF THE PREFERRED EMBODIMENT

The alloy of the present invention is a eutectic composition of nickel and chromium having a lamellar microstructure in which the lamellae are oriented in substantially the longitudinal direction of the alloy member or product, the major stress being applied in the longitudinal direction as in turbine blades, for optimum strength and high-corrosion resistance. The longitudinally oriented lamellar structure is preferably obtained by directional solidification of an alloy having a substantially eutectic composition of nickel and chromium. As shown in FIG. 1, the eutectic composition of the nickel-chromium system is located at about 50 weight percent nickel and 50 weight percent chromium. More particularly, the eutectic composition is 50±1 percent of chromium and 50±1 percent of nickel and may contain traces of incidental impurities such as iron. The melting temperature of the eutectic composition is approximately 1,345°C.

The phase diagram of the nickel-chromium system (FIG. 1) indicates that it is amenable to unidirectional solidification.

55 Both of the resulting phases (nickel-rich phase and chromium-rich phase) have widely spaced terminal solid solubility limits to provide for good corrosion resistance. The solubility is retrograde and second-phase precipitation is possible. When the eutectic composition solidification reaction is correlated with unidirectional solidification, there is produced a nickel-chromium composition with a regular lamellar structure and a minimum number of grain boundaries, as shown in FIG. 2. In order to obtain the properties having the desired combination of high strength, thermal stability, corrosion resistance, and creep resistance at elevated temperatures, control over the lamellar spacing is necessary.

Generally, the process for obtaining these properties in the binary alloy of nickel-chromium with a lamellar eutectic structure such as shown in FIG. 2, includes the following steps:

60 1. Cast a melt of an alloy of eutectic composition of nickel and chromium into a container-mold having a high melting point and holding the melt at a temperature above the melting point of about 1,350° C. for the alloy in a suitable furnace means such as a Bridgman furnace,

2. Lower the molten ingot through the lower end of the furnace at a constant velocity and into a quenching medium to produce a unidirectional lamellar structure; and

3. Cold work the resulting solidified ingot having a unidirectional lamellar structure until a reduction in area of from about 50 to 75 percent is achieved.

The resulting member has good strength up to about 1,400° F. When properly worked the alloy has a room temperature yield strength of about 300,000 p.s.i.

The following example is further illustrative of the present invention:

#### EXAMPLE

Specimens of a melt of a eutectic composition of nickel-chromium having 50 percent nickel and 50 percent chromium were cast into an alumina tubing having a one-quarter inch diameter and were held at temperature above the melting point of about 1,350° C. The particular type of furnace involved for this purpose was a Bridgman furnace. Other heating means such as the Czochralski furnace, molten zone passing, and directional casting, are satisfactory.

Each specimen was then lowered out of the molten zone of the furnace at a rate of about 0.39 inch per hour and into a body of water located below the furnace in order to quench the specimen into a solid rod, thereby causing unidirectional solidification. This technique gave a controlled linear movement of the liquid-solid interface and a controlled temperature gradient which result in the lamellar structure as shown in FIG. 2.

Compression and tensile specimens were prepared from the as-grown material and tested over a range of temperatures. The results of the tensile and compression tests are shown in tables I and II.

TABLE I.—TENSILE TEST DATA ON AS-GROWN Ni-Cr EUTECTIC

| Spec. Number: | Diameter (inches) | Gage length (inches) | Test Temp., °F. | 0.2% offset yield strength |        | Ultimate strength Lbs. | Elongation Inches | Reduction of Area Percent |
|---------------|-------------------|----------------------|-----------------|----------------------------|--------|------------------------|-------------------|---------------------------|
|               |                   |                      |                 | Lbs.                       | P.s.i. |                        |                   |                           |
| 1             | 0.099             | 0.560                | 75              | 432                        | 56,100 | 800                    | 103,900           | 0.167 29.8 0.079 36.4     |
| 2             | 0.098             | 0.560                | 1,460           | 319                        | 42,550 | 426                    | 56,800            | 0.153 27.8 0.065 56.0     |

TABLE II.—COMPRESSION TEST DATA ON Ni-Cr EUTECTIC

| Specimen Number: | Diameter (inches) | Percent work | Test Temp., °F. | Yield strength, p.s.i. |
|------------------|-------------------|--------------|-----------------|------------------------|
| 1                | 0.205             | 0            | 70              | 77,600                 |
| 2                | 0.205             | 0            | -220            | 155,000                |
| 3                | 0.140             | 80           | 1,470           | 48,500                 |
| 4                | 0.140             | 50           | 70              | 214,600                |
| 5                | 0.140             | 80           | 70              | 211,400                |
| 6                | 0.100             | 75           | -320            | 271,250                |
| 7                | 0.100             | 75           | 70              | 312,500                |
| 8                | 0.230             | 0            | 70              | 88,500                 |
| 9                | 0.230             | 0            | 1,470           | 31,600                 |

The material of the specimens was ductile enough to be cold worked and was swaged down to give rods with approximately 50 and 75 percent reduction in area. Compression specimens were made from the swaged rod.

Specimens were also tested for yield strength for the as-grown material as well as swaged rods and the results have been plotted (FIG. 3) as a function of  $d^{-1/2}$ , where  $d$  is the specimen diameter in inches. An extrapolation of the results shows that a potential yield strength of 1,000,000 p.s.i. may be possible upon refinement of the materials and the casting and working procedures of this invention. Extrapolating a bar having a cast diameter of 2.5 inches would have to be cold reduced to 0.2 inch to achieve this effect. The lamellae spac-

ing would then be reduced from the as-grown spacing of  $6 \times 10^{-5}$  inches to approximately  $5 \times 10^{-5}$  inch.

The Ni-Cr eutectic made for the above series of specimens was grown at a relatively slow rate of 0.39 inch per hour and the lamellae have fairly wide spacing. However, finer lamellae are obtainable by growing at a faster velocity. Thus, the yield strength would be enhanced and the amount of cold work required to reach a given strength is reduced. As shown in tables I and II the high-temperature tensile and compression yield strengths (about 35 k.s.i.) for the as-grown material are high enough for commercial applications such as turbine blades. Moreover, the mechanical properties at high temperatures are enhanced by cold work such as shown in compression specimen No. 3. (table II).

15 Evidence indicates that the lamellar structures are stable up to within a few degrees below the melting point. However, "coarsening" (thickening of the lamellae) occurs at temperatures close to the melting point. The lamellar structure is highly stable up to 100° or 200° below the melting point, and 20 the mechanical properties are retained even after extended heat treatment.

#### The Nickel-Rich Phase

The microstructure of the specimens resulting from the unidirectional growth is indicated in FIG. 2; that is, they have directionally solidified structure. The microstructure includes a continuous matrix which is the light-colored background and is composed of the nickel-rich phase. The dark, needlelike or thinner lamellae are the chromium-rich phase. Inasmuch as a two component system is involved, which rules out ternary hardeners for the nickel, an increase in the inherent strength of the matrix is obtained only through residual strain introduced by plastic deformations such as swaging or rolling.

In the directionally solidified eutectic the lamellar spacing is

therefore a very important factor in the overall matrix strength. As already indicated the lamellar spacing can be controlled directly to some extent during solidification and may be reduced by cold working.

45 Some comparative data on directionally solidified Ni-Cr alloys and a fully solution treated and aged superalloy are shown in FIG. 4. A typical composition of the alloy Rene 41 is 10 percent cobalt, 19 percent chromium, 3.2 percent titanium, 1.5 percent aluminum, 1.35 percent iron, 0.07 percent carbon, and the balance nickel which is usually sold under the trademark, Rene 41. In FIG. 4 the dependence of 0.2 percent yield 50 on cold work is shown for the Ni-Cr eutectic alloy and the Rene 41 alloy at room temperature and at 1,400° F. Both specimens were held for 1 hour at temperature prior to testing. The room temperature strength of the Rene 41 alloy increases by 80 K p.s.i. when rolled to 40 percent reduction in area. However, at 1,400° F. the strength of the worked alloy 60 returns to the room temperature strength of the unworked alloy, indicating that the strength of the worked alloy is primarily due to an increase in dislocation density which is removed by annealing at 1,400° F. The 1,400° F. performance would be even worse if it did not have dispersed particles of lamellae 65 generally of a nature similar to that of Ni-Cr alloy. Without this both the worked and unworked Rene 41 alloy would have far lower strength at 1,400° F.

On the other hand, the Ni-Cr alloy having the same amount 70 of cold work as the Rene 41 alloy has an increase of 15 K p.s.i. at room temperature which increase is attributable to the combined effects of dislocation density and to the reduction in the lamellar spacing. As evident from FIG. 4 at 1,400° F. the difference between the work and unworked Ni-Cr alloy samples is about 41 K p.s.i. which is about a factor of two greater

than the unworked strength. This is comparable to the difference between the two Rene 41 specimens at this temperature. It is believed therefore that the lamellar spacing in the Ni-Cr alloy does form an effective barrier to moving dislocations. Moreover, the effectiveness of the lamellar structure would be greatly improved if the lamellar spacing were decreased by, say, an order of magnitude.

#### The Chromium-Rich Phase

The lamellae are composed of a chromium-rich phase and contribute substantially to the strength of the composite where the thickness of the lamellae is in the range of sub-micron to micron dimensions. A reduction in the chromium lamellae thickness by controlled solidification results in substantial increases in the strength properties.

As shown in FIG. 1 the solidus slope of the chromium-rich phase is very steep and retrogrades near the eutectic isotherm, sweeping from a composition of about 30 percent of Ni downwardly toward a very much lower value of about a few percent at room temperature. The chromium-rich phase is therefore more highly supersaturated with respect to the nickel-rich phase.

#### Creep Behavior

In addition to the foregoing tests, specimens of Ni-Cr eutectic alloys were tested for creep resistance at 1,400° F. (760° C). The stress-rupture data are summarized in FIG. 5 where three sets of data are represented. The effect of directional solidification is quite pronounced. An increase of close to two orders of magnitude in time to failure for a given stress is obtained by the lamellar alloy over the cast alloy which represents the nickel-rich matrix in the eutectic composite. The intermediate curve is for partially lamellar and partially dendritic material, where the full benefit of aligned composite structure is not realized.

Further, creep tests were performed on the Ni-Cr eutectic alloy specimens prepared in accordance with this invention,

Cr-40 Ni alloys, both "hi" and "low" carbon. It is evident that the Ni-Cr eutectic alloy has creep resistance properties that are highly satisfactory as well as being superior to the 60 Cr-40 Ni alloys.

#### 5 Corrosion Resistance

In the past it has been found that at least 12 percent chromium in Ni-Cr alloys was necessary to give fair corrosion resistance at high temperature. The mechanical properties of this alloy are improved as the percentage of chromium is reduced, but at the same time the corrosion resistance is lessened. The corrosion resistance of the 50-50 percent Ni-Cr eutectic alloy is excellent and the mechanical properties are outstanding as a consequence of the lamellar structure. As cast specimens of Ni-Cr eutectic alloys were subjected to an accelerated 500 hour combustion test at 1,500° F. in Diesel fuel oil containing 6.9 percent sulfur. The specimens were first dipped in a molten eutectic salt bath of magnesium and sodium sulfates which provide a representative fuel slag coating and accelerate the tests at this high-sulfur level. To maintain the sulfate stability, the partial pressures of SO<sub>2</sub> and SO<sub>3</sub> were artificially increased to 2,000 and 70 p.p.m., respectively. As shown in FIG. 7, the corrosion resistance of the Ni-Cr eutectic alloy is superior to several high-temperature superalloys and stainless steels previously used for turbine blades, such as Inco 713-C, Udiment 700 and 500 alloys. The Ni-Cr alloy was also compared with other known corrosion resistant alloys such as Hastelloy-X and type 310 stainless steel. Specimens of the Ni-Cr eutectic alloy were examined for penetration in both this sulfidation and also in simple oxidation tests, and these tests showed that the chromium-rich lamellae very effectively block penetration. Oxidation pits which penetrated the first nickel-rich phase were stopped effectively by the first chromium lamellae they encountered.

Typical analyses for the indicated nickel-base alloys are listed in table IV.

TABLE IV

| Alloy       | C    | Cr    | Co | Mo   | Cb  | Ti  | Al  | B     | Zr   | Fe   | Ni    | W   | Mn   | Si   |
|-------------|------|-------|----|------|-----|-----|-----|-------|------|------|-------|-----|------|------|
| INCO713C    | 0.12 | 12.5  |    | 4.2  | 2.0 | 0.8 | 6.1 | 0.012 | 0.10 |      | Bal.  |     |      |      |
| UDIMET700   | 0.08 | 15.0  |    | 18.5 | 5.2 | 3.5 | 4.3 | 0.03  |      |      | Bal.  |     |      |      |
| UDIMET500   | 0.07 | 19.0  |    | 19.0 | 4.2 | 3.0 | 3.0 | 0.007 | 0.05 |      | Bal.  |     |      |      |
| UDIMET520   | 0.05 | 19.0  |    | 12.0 | 6.0 | 3.0 | 2.0 | 0.005 |      |      | Bal.  | 1.0 |      |      |
| HASTELLOY X | 0.10 | 22.0  |    |      | 9.0 |     |     |       |      | 18.5 | Bal.  | 0.5 | 0.50 | 0.50 |
| 310SS       | 0.25 | 24.26 |    |      |     |     |     |       |      | Bal. | 19.22 | 2.0 | 1.5  |      |

<sup>1</sup> Maximum.

compared with data for a commercially cast 60 percent chromium-40 percent nickel alloy. The analysis of the commercially cast alloys having "Lo carbon" and "Hi carbon" as well as the Ni-Cr eutectic alloy used for comparison are shown in table III.

TABLE III

Chemistries of two International Nickel Co. 60 percent Cr-40 percent Ni alloys, and of the least pure Ni-Cr eutectic (all other elements < 0.01 percent)

|        | Fe   | Si   | C    | Mn   |
|--------|------|------|------|------|
| "Lo C" | 0.72 | 0.9  | 0.01 | —    |
| "Hi C" | 3.45 | 1.17 | 0.14 | 0.32 |
| Ni-Cr  | 0.1  | 0.02 | 0.01 | 0.05 |

The creep-rupture test results are plotted in FIG. 6, and in view of the purity of the Ni-Cr eutectic alloy, it demonstrates excellent performance compared with the two 60 percent Cr, 40 percent Ni alloys of "Lo" and "Hi" carbon content as set forth in table III. Here again it is evident that a fine, well-controlled, lamellar structure provides a highly satisfactory creep resistance property in the Ni-Cr eutectic alloy.

Moreover, the creep-rupture tests for the Ni-Cr eutectic alloy are included in FIG. 6 to compare the alloy with the 60

#### CONCLUSION

The overall thermal stability of the lamellar structure of the Ni-Cr eutectic alloy was demonstrated to be satisfactory. Thus, the lamellar structure of the alloy exhibits little change in creep resistance after exposure for 15 hours at 15 K p.s.i. and 1,500° F. The excellent lamellar structure remained unchanged. Moreover, the improvement in the yield strength of the cold-worked Ni-Cr eutectic alloy has been shown to be generally superior to prior known alloys which were conventionally regarded as highly satisfactory. In addition the corrosion resistance of the Ni-Cr eutectic alloy is better than or equivalent to the best prior used alloys having acceptable corrosion resistance properties.

Accordingly, the Ni-Cr eutectic alloy having a lamellar eutectic microstructure is suitable for use in many applications including such diverse uses as in watch springs and turbine blades. In the latter environment the alloy more than satisfies the life time requirement to which turbine blades are subjected at temperatures of up to 1,400° F. and at the same time the alloy demonstrates satisfactory resistance to corrosion without sacrificing strength, thermal stability, and creep resistance properties.

Although the best known embodiment of the invention has been described in detail, it is understood that the invention is not limited thereto or thereby.

What is claimed is:

1. A member of a directionally solidified high-temperature alloy having high creep-rupture properties, thermal stability and resistance to corrosion and consisting of a eutectic composition of  $50\pm1$  percent nickel and  $50\pm1$  percent chromium, and the member having a metallurgical microstructure comprising oriented chromium-rich lamellae in a nickel-rich matrix.

2. A member of the alloy of claim 1 which has been cold worked to provide a reduction in area of about from 50 to 75 percent.

3. A turbine blade comprising a directionally solidified eutectic composition of  $50\pm1$  percent nickel and  $50\pm1$  percent chromium, and having a metallurgical microstructure comprising oriented chromium-rich lamellae in a nickel-rich

matrix.

4. A process for producing a member comprising a eutectic composition of nickel and chromium which comprises (1) casting a melt of eutectic alloy of  $50\pm1$  percent nickel and  $50\pm1$  percent chromium into a mold having a high-melting point and holding the melt at a temperature above the melting point of about  $1,350^{\circ}\text{C}$ . for the alloy in a suitable furnace, (2) lowering the melt out of the furnace at a constant velocity and into a quenching medium to produce an ingot having a unidirectional lamellar structure, and (3) cold working the ingot until a reduction in area of from about 50 to 75 percent is achieved.

\* \* \* \* \*

15

20

25

30

35

40

45

50

55

60

65

70

75